

Nov. 25, 1924.

1,516,804

E. L. WILKE ET AL

## METHOD AND APPARATUS FOR GAUGING CASTINGS

Filed April 5, 1923



Fig. 1.



Fig. 2.

Erwin L. Wilke  
James O. Johnston  
by Clegg, Clegg, Atty.

## UNITED STATES PATENT OFFICE.

ERWIN L. WILKE, OF HAMMOND, AND JAMES O. JOHNSTONE, OF EAST CHICAGO, INDIANA, ASSIGNORS TO METALS REFINING COMPANY, OF HAMMOND, INDIANA, A CORPORATION OF INDIANA.

## METHOD AND APPARATUS FOR GAUGING CASTINGS.

Application filed April 5, 1923. Serial No. 629,985.

To all whom it may concern:

Be it known that we, ERWIN L. WILKE and JAMES O. JOHNSTONE, both citizens of the United States, residing, respectively, at 5 Hammond and East Chicago, in the county of Lake and State of Indiana, have invented new and useful Improvements in Methods and Apparatus for Gauging Castings, of which the following is a specification.

10 This invention relates to a method and apparatus for determining the highest grade of castings from any given metal.

In order to gain a clear understanding of our invention, the following explanation 15 is made. Antimonial lead is used for castings of all kinds. Most of such castings are made in metallic molds, and some castings are more intricate than others; namely, the metal must be flowed fully and completely 20 into fine lines or portions. Such intricacies involve not only clean metal but also observance of certain conditions. In many castings failure to observe such conditions has led to the belief that casting 25 failures were due to dirty metal, whereas this is not essentially a fact.

Take for example the casting of type for printing presses and more particularly 30 type used in printing the daily metropolitan newspapers. The type must be made of metal of such hardness as to withstand the running off of many thousand copies of a single edition. A metal having such 35 property is difficult to pour under the conditions existing heretofore, with the result that imperfect castings were made, resulting in loss of material as well as time and labor. Furthermore, when running off thousands of copies of a single edition, 40 the type cast under the heretofore existing conditions would not stand up and after a certain number of copies had been run off the type became very badly worn with the 45 result that the balance of the copies were blurred and therefore not saleable.

Another instance of the conditions heretofore may be mentioned, and that is the 50 coating of electric cable with an outside covering of a lead alloy. The producer of the metal often is required to guarantee that the metal will produce a coating of a certain thickness throughout the entire length of the cable, the latter varying in relatively long lengths, or to guarantee that

the metal will not crack on winding the 55 cable on a reel. In the event of failure of this metal in any part of the length of the cable, whether at the beginning, end, or any intermediate part, the manufacturer of the 60 cable would take advantage of the guarantee by way of penalty in the contract with the result that great loss of money was suffered by the maker of the metal.

So it is in other casting operations, where 65 fineness of product is required great loss of material, time, and labor resulted in obtaining imperfect castings, due to a number of conditions which it is the object of our invention to overcome.

We have found by actual experiment and 70 demonstration that, in order to produce perfect castings, it is absolutely necessary to take into account the temperature of the metal as poured and the temperature of the 75 mold into which the metal is poured. When making castings of a certain grade, the best results are secured when the metal and mold temperatures bear a certain ratio to each other, and the same holds true with respect to the kind of metal being used. To 80 determine these temperature ratios required for different grades of castings in order that the best castings may be secured of the different grades, we make an apparatus such as shown in the accompanying drawings. In these—

Fig. 1 is an end view of a mold provided with a mold cavity made in accordance with our invention; and

Fig. 2 is an enlarged view showing the 90 design of said cavity.

As shown in the drawings, the mold comprises two separable mold members A, B, one of which has an outwardly projecting part C for supporting the mold in the position of use. Said mold members are clamped together in any suitable manner, as by two C-clamps D, D in Fig. 1.

The inner face of the mold member A is provided with the mold cavity of our invention. This is given a design including all varieties of casting sections, that is, heavy and thin sections, fine and coarse lines, intersecting lines, etc. As shown in Fig. 2, the design comprises a main vertical 105 groove E of a uniform section throughout its length.

On each side of the main groove E is a

set of downwardly inclined branch grooves F, G, and H. In both sets, the branch grooves have substantially the same extent of inclination and are alike. Said branch 5 grooves have their greatest section at their entrance into the main groove E and diminish in section toward their outer ends, where they become fine lines. The grooves F to H on one side of the main groove E 10 are above the corresponding ones on the opposite side so that the filling of a branch groove on one side of said main groove will not be at the expense of the corresponding one on the opposite side.

15 Each set of branch grooves F, G, and H are connected by a vertical groove I. This terminates in the lower groove F, intersects and crosses the middle and top grooves G and H. It extends above said top groove 20 H, as shown in Fig. 2. Said grooves I are substantially uniform in section throughout their lengths, as shown. In addition, each set of branch grooves F, G, and H have vertical grooves J, K, and L, one for each 25 branch groove. These vertical grooves decrease in section toward their upper ends and there terminate short of the branch grooves above in fairly fine lines, as shown in Fig. 2.

30 The upper end of the mold has a filling recess M, which communicates with a smaller recess N, the latter opening directly into the upper end of the main groove E. As shown in dotted lines in Fig. 1, each of the mold 35 members A, B is provided with a part of this filling recess M. Except for this recess being in both mold members, the rest of the mold cavity is in the mold member A and not in the one B, in the particular design 40 and structure shown.

The mold member A, in addition to the mold cavity described, is also provided with a chamber O adapted to be filled with mercury and into which is inserted a thermometer 45 or other heat registering gauge P.

45 The mold or apparatus is used as follows. The mold members A, B are clamped together, and their temperature raised to a predetermined point by the application of 50 heat, as by gas burners. Molten metal of the kind to be tested is then poured into the mold cavity through the filling recesses M, N. The temperature of the molten metal at the time of pouring is determined and a record kept of it. To align the mold members 55 A, B and hold them in that relation when clamped together, dowel or like pins Q, Q are provided.

The main groove E being in line with the 60 filling recesses M and N and having a substantially uniform section throughout its length will fill first and will be the easiest part of the cavity to fill. The other grooves will fill in the order of their location and 65 shape. The bottom grooves F, F will natu-

rally fill before the ones above, and the molten metal will rise in the vertical grooves J and adjacent portions of the ones I from the bottom grooves F. Filling of the outer ends of the grooves F will be rendered somewhat 70 difficult by reason of the fact that they taper off in dimension in that direction and become very fine at their extreme outer ends. Gravity, however, assisting the filling will play its part, whereas gravity will not aid 75 in filling the fine upper ends of the grooves J. Next to fill from the main groove E are the upper grooves G, and a part of the vertical groove I on each side thereof will fill from that groove and meet the molten metal 80 in the groove from the groove F therebelow. The grooves K will fill in the same manner as the ones J, and so on throughout the entire shape of the mold cavity. To permit the escape of air, vent lines are provided in 85 connection with the several grooves, as shown in Fig. 2, and these lines for convenience are all marked a'.

We have given all of the grooves of the mold cavity certain numerical valuations 90 based on 100% and in such proportions thereof as indicate the difficulties the metal encounters in filling the various parts of the cavity, depending on the fineness and location of the grooves. For illustration, we 95 have given the main groove E a rating of 10; while for the portion of each branch groove F, G and H at the main groove E, a rating of 1; for the portions of these branch grooves between the vertical grooves 100 I and J, a rating of 2; and for the outer end portions of these branch grooves beyond the vertical grooves I, a rating of 3, as marked on Fig. 2. For each vertical groove J, K, and L, we give a rating of 4, 105 because it is more difficult to fill these grooves than the other groove parts mentioned, and for each portion of the groove I, a rating of 5, because of the fact that that groove is likely to fill from both top and 110 below with a chance of trapping air between the filling parts of the column. Adding the ratings of the various grooves on each side of the main groove will give 90, 45 for each side of the main groove E. Adding 115 the rating for the main groove E to the above figure will total 100, indicating the full percentage for the entire mold cavity.

Starting with the metal being tested at a 120 certain temperature and with the mold at a certain temperature and producing a casting with the device described, will show on inspection of the casting just what difficulties were encountered in filling the various parts of the grooves. If any imperfections are 125 found, it is apparent that either the temperature of the mold or the temperature of the metal needs changing. The temperature of the mold may be raised or lowered as the test may require and another casting made 130

which on inspection will show the actual conditions encountered. By making the series of tests with the metal at a given temperature and starting with the mold at one temperature and raising it throughout the entire series of tests, will determine the best grade of castings that can be obtained when the mold and metal are at certain given temperatures.

10 Likewise, tests can be made by keeping the mold at a given temperature and varying that of the metal being poured. In this way the best grade of castings can be determined and thus the manufacturer of the metal has some means to determine beforehand just what will produce the best grade of castings for the different industrial uses to which the metal is put. Thus, in connection with the printing of newspapers the method and device of our invention can determine at what heat the metal for the type should be poured and what the mold temperature should be to gain the best results for any number of copies of an edition that 20 may be run off without having the type fail. In the same way the invention and apparatus can determine at what temperature the mold metal can be best used for coating electric cables, and so on.

30 While we have shown and described herein in detail an apparatus or mold for practicing the method of our invention, we, of course, do not wish to be limited to the exact details of structure thereof because they 35 may be variously changed and modified without departing from the spirit and scope of our invention, nor do we wish to be limited to the particular application of our invention as herein described.

40 We claim as our invention:

1. The method of determining the highest grade of castings from any given metal, which consists in determining the mold and metal temperatures required for such castings.

45 2. The method of determining the highest grade of castings from any given metal, which consists in determining the mold and metal temperatures required for such castings by pouring the molten metal into a mold and keeping either the molten metal or the mold at a substantially constant temperature while varying the temperature of the other.

50 3. The method of determining the highest grade of castings from any given metal, which consists in determining the mold and metal temperatures required for such castings by pouring the molten metal at varying temperatures into a mold kept at a substantially constant temperature.

55 4. The method of determining the highest grade of castings from any given metal, which consists in determining the mold and metal temperatures required for such cast-

ings by pouring the molten metal at a substantially constant temperature into a mold at various temperatures.

5. The method of determining the highest grade of castings from any given metal, 70 which consists in determining the mold and metal temperatures for such castings and pouring the molten metal into a mold cavity having a design including a variety of casting sections.

75 6. The method of determining the highest grade of castings from any given metal, which consists in determining the mold and metal temperatures for such castings and pouring the molten metal into a mold cavity 80 having a design including a variety of casting sections, that is, heavy and thin sections, fine and coarse lines, intersecting lines, etc.

7. The method of determining the highest grade of castings from any given metal, 85 which consists in determining the mold and metal temperatures for such castings and pouring the molten metal into a mold cavity 90 having a design including a variety of casting sections and having a table of values for different parts of said design based on the intricateness thereof and difficulty to fill, which values when all perfect total 100%.

8. A mold for the purpose described, having a mold cavity of a design representing 95 a variety of casting sections.

9. A mold for the purpose described, having a mold cavity of a design representing 100 a variety of casting sections, including heavy and thin sections, fine and coarse lines, intersecting lines, etc.

10. A mold for the purpose described, having a mold cavity of a design comprising a main groove having a substantially uniform section throughout its length and opening directly into the filling opening of the mold, branch grooves on opposite sides of said main groove and arranged at angles thereto, said branch grooves opening into said main groove at their inner ends and decreasing in section toward their outer ends, and additional grooves on opposite sides of said main groove and transverse to said branch grooves, said additional grooves opening into their associate branch grooves 110 between the ends of the latter.

11. A mold for the purpose described, having a mold cavity of a design comprising a main groove having a substantially uniform section throughout its length and opening directly into the filling opening of the mold, branch grooves on opposite sides of said main groove and arranged at angles thereto, said branch grooves opening into said main groove at their inner ends and decreasing in section toward their outer ends, and additional grooves on opposite sides of said main groove and transverse to said branch grooves, said additional grooves opening into their associate branch grooves 120 115 125 130

- between the ends of the latter and arranged with a branch groove on each side of said main groove intersecting at least two branch grooves.
- 5 12. A mold for the purpose described, having a mold cavity of a design comprising a main groove having a substantially uniform section throughout its length and opening directly into the filling opening of
- 10 the mold, branch grooves on opposite sides of said main groove and arranged at angles thereto, said branch grooves opening into said main groove at their inner ends and decreasing in section toward their outer ends,
- 15 additional grooves on opposite sides of said

main groove and transverse to said branch grooves, said additional grooves opening into their associate branch grooves and arranged with a groove on each side of said main groove intersecting at least two branch grooves, and table of values for said grooves based on the sections thereof and the difficulty of filling, which values when all perfect total 100%.

20 In testimony that we claim the foregoing as our invention, we affix our signatures, this 31 day of March, A. D. 1923.

ERWIN L. WILKE.  
JAMES O. JOHNSTONE.